

Aug. 20, 1940.

C. F. BALDWIN ET AL

2,212,139

PIEZOELECTRIC QUARTZ ELEMENT

Filed March 18, 1936

FIG. 1.



4 Sheets-Sheet 1

FIG. 2.



FIG. 3.



FIG. 6.



FIG. 4.



FIG. 5.



INVENTORS  
Samuel A. Bokovoy  
Charles F. Baldwin

BY

ATTORNEY

Aug. 20, 1940.

C. F. BALDWIN ET AL.

2,212,139

PIEZOELECTRIC QUARTZ ELEMENT

Filed March 18, 1936

4 Sheets-Sheet 2

FIG. 7.

ZERO OR OTHER LOW TEMPERATURE COEFFICIENT  
OF FREQUENCY CURVES FOR THICKNESS  
OSCILLATORS AND RESONATORS  
V-CUT



INVENTORS  
Samuel A. Bokovoy  
Charles F. Baldwin

BY   
ATTORNEY

Aug. 20, 1940.

C. F. BALDWIN ET AL

2,212,139

PIEZOELECTRIC QUARTZ ELEMENT

Filed March 18, 1936

4 Sheets-Sheet 3

FIG. 8.

FREQUENCY CONSTANTS  $K^m$  AND  $V^m$   
FOR V-CUT QUARTZ  
THAT FALLS ALONG THE ZERO TEMPERATURE  
COEFFICIENT CURVES SHOWN BY  $\pm 10^\circ$  CURVES  
OF FIG. 7.



INVENTORS  
Samuel A. Bohovoy  
Charles F. Baldwin

BY

*J. J. Jaff*

ATTORNEY

Aug. 20, 1940.

C. F. BALDWIN ET AL  
PIEZOELECTRIC QUARTZ ELEMENT

2,212,139

Filed March 18, 1936.

4 Sheets-Sheet 4



FIG. 9.

INVENTORS  
Samuel A. Bokovoy  
Charles F. Baldwin

BY

ATTORNEY

## UNITED STATES PATENT OFFICE

2,212,139

## PIEZOELECTRIC QUARTZ ELEMENT

Charles F. Baldwin, Schenectady, N. Y., and  
Samuel A. Bokovoy, Audubon, N. J., assignors  
to Radio Corporation of America, a corporation  
of Delaware

Application March 18, 1936, Serial No. 69,496

21 Claims. (Cl. 171—327)

This invention relates to the piezoelectric art, particularly to the cutting of quartz piezoelectric elements and has special reference to the manufacture of piezoelectric quartz elements of the type possessing a natural mode of vibration which is a function of thickness. It is a continuation in part of application Serial Number 721,675 to Charles F. Baldwin and Samuel A. Bokovoy, filed April 21, 1934, and assigned to the same assignee 10 as the instant case.

It is known to those skilled in the art that an "X-cut" quartz piezoelectric element (that is to say, one cut in the form of a rectangular plate having its electrode faces so orientated 15 with respect to the mother crystal that its thickness dimension is along an electric axis and its length or width along either the optic axis or a mechanical axis), will exhibit variations in frequency when subjected to temperature 20 changes. The same phenomenon obtains if the crystal is Y-cut, i. e., if the thickness dimension of the element is along a mechanical axis and its length or width along either an electric axis or the optic axis.

In order to compensate for variations in frequency resulting from variations in temperature, all sorts of auxiliary frequency control apparatus have heretofore been employed. Obviously a piezoelectric-element possessing a zero temperature coefficient of frequency will not require an elaborate thermostatically controlled constant temperature cabinet to maintain a constant frequency of oscillation.

An object, therefore, of the present invention 35 is to provide a quartz piezoelectric element which shall exhibit a zero temperature coefficient of frequency.

Another object of the invention is to provide a quartz-piezoelectric element which shall exhibit 40 a zero or some other desired low temperature coefficient of frequency when vibrated at a frequency which is a function of its thickness dimension.

Another object of the invention is to provide 45 a process for so cutting a piezoelectric element that its fundamental frequency will be high relative to its thickness.

Another object of the invention is to provide 50 a simple, accurate and efficient mode of procedure in the cutting of quartz crystals to eliminate as far as possible any uncertainties with regard to the frequency, the temperature coefficient of frequency and other operating characteristics of the finished element.

Still another object of the invention is to provide 55 a process for so cutting piezoelectric crystals that there will be minimum wastage due to the production of non-usable elements.

Other objects and advantages will be apparent 60 and the invention itself will be best understood

by reference to the following specification and to the accompanying drawings, wherein:

Figure 1 is a plan view of a natural or "mother" quartz crystal, the optic (Z) axis of which is perpendicular to the plane of projection, the 5 relative location of the apex, major and minor apex surfaces, an electric (X), a mechanical (Y) axis, a reference W axis and a reference  $Y+\theta$  axis being here illustrated as an aid to a clear understanding of the system of orientation followed in producing quartz piezoelectric elements 10 in accordance with the invention.

Fig. 2 shows in outline and in perspective a piece of natural quartz having a section cut and divided to provide a rough bar having top and 15 bottom surfaces lying in planes which are normal to the Z-axis and its long edges parallel to a W-axis which is  $20^\circ$  removed from an X-axis.

Fig. 3 is an elevational view looking in the direction of the arrow of Fig. 2 showing the 20 position of two blanks cut from the bar of Fig. 2, one of these blanks is tilted towards parallelism with the plane of a major apex surface of the mother-crystal and the other toward parallelism with the plane of a minor apex surface of the 25 mother crystal.

Fig. 4 shows the left hand blank of Fig. 3 removed and trimmed, the plane of projection being perpendicular to the plane of the paper.

Fig. 5 shows the right-hand blank of Fig. 3, 30 removed and trimmed.

Fig. 6 is a cross-sectional view taken on the line Y—Y of Fig. 1 showing the rotation of the blanks about a  $Y+\theta$  reference axis of a mother crystal and with respect to the major and minor 35 apex surfaces thereof.

Fig. 7 is a chart showing the correlation between certain angles  $W^n-V^n$ , and  $W^m-V^m$ , required to achieve a thickness-mode oscillator having a zero or other low temperature coefficient 40 of frequency.

Fig. 8 is a chart of the frequency constants ( $K^n$  and  $K^m$ ) peculiar to zero temperature coefficient thickness-mode crystals.

Fig. 9 is a chart indicative of the characteristics of quartz plates rotated throughout the entire  $360^\circ$  scale about the Z-axis.

As above indicated the present invention contemplates and its practice provides a quartz piezoelectric element which exhibits a zero temperature coefficient of frequency, or a temperature coefficient of either sign and of a desired low value, when vibrated at a frequency which is a function of its thickness dimension.

This desired operating characteristic obtains, 55 in accordance with the invention, by reason of a rotation or inclination of the principal electrode faces of the element about any of certain  $Y+\theta$  axes. Each of these  $Y+\theta$  axes is normal to a W-axis, which W-axes lie in certain later speci- 60

fied ranges in the X-Y plane normal to the Z-axis.

The direction of rotation or "tilt" is away from parallelism with the Z-axis and may be toward 5 parallelism with the plane of a major or a minor apex surface of the mother crystal. The exact angle of rotation about the selected  $Y+\theta$  axis depends upon the direction towards which the 10 electrode faces of the element are directed and also upon the exact temperature coefficient of frequency desired.

Certain frequency constants ( $K$ ) are given for each W-axis or angle so that it is possible to know in advance the substantially exact thickness dimension required to achieve a desired thickness-mode frequency. The temperature coefficients are also given for each angle of rotation in a standard frequency range.

Since the present invention involves a system 20 of orientation in which (a) the major and minor apex surfaces of the mother-crystal are employed as reference planes and (b) certain W-axes and (c) certain  $Y+\theta$  axes are employed as reference axes, it is first necessary to identify these planes 25 and axes.

As to (a), referring to Figs. 1 and 2 of the drawings and having in mind that all unbroken quartz crystals are hexagonal bi-pyramids, it will be seen that certain of the terminal surfaces of 30 the quartz extend to the apex of the pyramid. These surfaces are designated M and are the major apex surfaces. Those terminal surfaces which do not touch the apex are designated N and are the minor apex surfaces of the mother-crystal. 35 Occasionally a mother crystal will be found in which more than three of the apex or "cap" faces extend to the tip of the pyramid; other crystals may have their pyramid ends broken off. No confusion, however, need exist as to 40 the virtual location of the major and minor apex faces of a broken or otherwise abnormal crystal providing that the side faces  $m$  and  $n$ , or one of them, is intact for it will be apparent from an inspection of Fig. 2 that those side edges of 45 the mother crystal which approach each other in the direction of its ends terminate in a major apex face, while those which diverge in this direction terminate in a minor apex face. This is so in the case of both "left-hand" and "right-hand" quartz.

As to (b), Fig. 1 is marked to show an electric, X-axis and an adjacent mechanical or crystallographic, Y-axis. The optic or Z-axis, marked in Fig. 2, is perpendicular to the plane of projection in Fig. 1. The W-axes lie between an X-axis and an adjacent Y-axis in the X-Y plane, i. e. in a plane normal to the Z-axis. There are a substantially infinite number of such W-axes; however, the present invention contemplates the 50 use as reference axes only those W-axes which in intersecting any reference X-axis form a W-angle therewith of from substantially  $13^\circ$  to substantially  $29^\circ$  or from substantially  $15^\circ$  to substantially  $29^\circ$ , depending upon the direction of tilt. In Fig. 1, but one W-axis is marked, it forms a W-angle of  $20^\circ$  with that X-axis which is designated X-X.

As to (c), there is a  $Y+\theta$  axis for each W-axis, each is normal to its W-axis and normal to the Z-axis. It is about a  $Y+\theta$  axis that the element is rotated or tilted to achieve a desired temperature coefficient of frequency and frequency constant.

It may here be noted that a W-axis  $30^\circ$  removed from an X-axis will coincide with a Y-

axis, hence its  $Y+\theta$  axis will coincide with another one of the X-axes. When a crystal blank is rotated about such a  $Y+\theta$  axis it is being rotated about this "another one" of the X-axis. Such orientation is not within the purview of 5 the present invention but forms the subject matter of copending application Serial Number 62-300, filed February 4, 1936, in the name of the present applicants and assigned to the same assignee as the instant case.

In order to produce a quartz piezoelectric element or "plate" having a predetermined low-temperature coefficient, a suitable angle of orientation (angle W) with respect to an X-axis, and a coordinated angle representing the inclination of the electrode (i. e. "top" and "bottom") faces must be chosen. This latter angle will be referred to generally as the "V-angle" and more specifically as the "V<sup>m</sup> angle" or the "V<sup>n</sup> angle" 15 as determined by the direction of rotation, i. e., 20 whether towards parallelism with the plane of a major apex surface ( $m$ ) or a minor apex surface ( $n$ ) of the mother crystal.

Referring now to Fig. 7 which shows the correlation between the temperature coefficient and 25 the angles W and V. In this chart an X-axis and an adjacent Y-axis are indicated by the vertical, correspondingly designated, lines and the space or region therebetween is calibrated in degrees from the X-axis, the calibrations being 30 along the horizontal line which intersects the centrally marked optic axis, Z. In agreement with the previously given definition a line extending at right angles at any point along this line will coincide with a W-axis. Horizontal line  $n-n$  extends from a point substantially  $13^\circ$  from the X-axis to within  $1^\circ$  of the Y-axis (i. e.  $29^\circ$  from the X-axis) and horizontal line  $m-m$  extends from a point substantially  $15^\circ$  to  $29^\circ$  from the X-axis, both lines  $n-n$  and  $m-m$  marked preferred limits within which a reference W-axis 35 may be selected.

It will be noted that there are two scales marked along the line representing the X-axis. That scale which reads in an "upward" direction from 40  $0^\circ$  represents a rotation of the electrode faces of the element about its  $Y+\theta$  axis in a direction away from parallelism with the Z-axis and towards parallelism with the plane of a minor apex surface of the mother-crystal, the calibrations 45  $V^n$  being in degrees from parallelism ( $0^\circ$ ) with the Z-axis. That scale which reads in a "downward" direction from  $0^\circ$  represents a rotation of the electrode faces of the element about its  $Y+\theta$  axis in a direction away from parallelism with the Z-axis and towards parallelism with the plane of a major apex surface of the mother-crystal; the calibrations  $V^m$  like those of  $V^n$  being in degrees from parallelism with the optic 50 axis.

Now, having in mind that there is a  $Y+\theta$  axis for, and normal to, each W-axis, then, from an examination of this Fig. 7 it will be seen that for each W-axis which forms an angle (W) with an X-axis within the  $13^\circ-29^\circ$   $n-n$  range, or  $15^\circ-29^\circ$   $m-m$  range, there is a definite angle of rotation ( $V^n$  or  $V^m$ ) required to achieve a desired temperature coefficient of frequency. For example, assuming that a piezoelectric element is required which shall exhibit a substantially zero temperature coefficient of frequency, assuming further (for reasons later set forth) that such element is to be so cut that its electrode faces are tilted in a direction away from parallelism with the Z-axis and towards parallelism with the plane of 55

5 a minor apex surface of the mother-crystal. Now, selecting any W-angle within the limits  $n-n$ , say  $20^\circ$  (read along the line which intersects the Z-axis), then, the correlated  $V^n$  angle of rotation of the electrode surfaces of the element about the  $Y+\theta$  axis is substantially  $36.5^\circ$ , this latter reading being obtained by observing at what point on the upper left hand scale a line will fall projected at right angles to a  $20^\circ$  W-axis 10 from a point (p) at which the said W-axis crosses the zero temperature-coefficient line.

An element exhibiting a zero temperature coefficient of frequency may likewise be achieved by tilting the electrode surfaces about a  $Y+\theta$  axis 15 towards parallelism with the plane of a major apex surface. Thus, assuming as in the above example that a  $20^\circ$  W-axis is selected, then, reading the lower left-hand scale at the point (p') where a  $20^\circ$  W-axis crosses the zero temperature 20 coefficient line it will be seen that the correlated  $V^m$  angle of rotation is substantially  $43^\circ$ .

The curves of Fig. 7 show clearly that the invention is not limited in its scope to the cutting of piezoelectric plates having an exactly zero temperature coefficient of frequency. For certain 25 uses the characteristic to be sought is a definite positive or negative temperature coefficient. Such crystal elements have great utility in oscillator circuits which inherently have certain 30 temperature coefficients of frequency irrespective of the crystal frequency control therefor. Thus it becomes advantageous at times to use a crystal control element having a temperature coefficient of frequency which is of opposite sign to, and substantially compensates for, the natural 35 temperature coefficient of frequency of an oscillator network per se.

To determine the  $V^n$  or the  $V^m$  angle of rotation required to achieve a piezoelectric element 40 having a particular temperature coefficient of frequency the left-hand scale of Fig. 7 should be read at the point where the selected W-angle crosses the line specific to the temperature coefficient desired. But three temperature coefficient 45 curves are marked in each of the charts of Fig. 7. There is a zero temperature coefficient curve (the center curves, each marked " $\pm 0$ ") for each direction of tilt. The curves on opposite sides of the "zero line" of the upper chart embrace the  $W^n$  and  $V^n$  angles required to achieve 50 an element exhibiting a temperature coefficient of frequency within  $+15$  cycles and  $-15$  cycles, respectively, per million, per degree centigrade. The curves on the opposite sides of the "zero line" of the lower chart embrace the  $W^m$  and  $V^m$  angles required to achieve an element exhibiting 55 a temperature coefficient of frequency within  $-5$  cycles and  $+5$  cycles, respectively, per million, per degree centigrade. Since all of the curves of the 60 respective charts of Fig. 7 are substantially parallel one with another, it is obvious that other curves representative of other temperature coefficients of frequency may be derived from the ones illustrated.

65 Before proceeding with the cutting of the blanks it is first preferable to determine of what thickness the finished element must be to achieve a desired fundamental thickness-frequency. This is simply accomplished in accordance with 70 the formula

$$t = \frac{K^n}{f} \quad (1)$$

or

$$t = \frac{K^m}{f} \quad (2)$$

where,  $t$  is the required thickness in mils of an inch  $K^n$  is a frequency constant which varies for each W-axis, when the direction of tilt of the element (about its  $Y+\theta$  axis) is towards parallelism with the plane of a minor apex surface of the mother-crystal.  $K^m$  is a frequency constant which varies for each W-axis, when the direction of tilt of the element about its  $Y+\theta$  axis is towards parallelism with the plane of a major apex surface of the mother-crystal, and  $f$  is the desired fundamental thickness-frequency, expressed in megacycles.

The frequency constants  $K^n$  and  $K^m$  are shown in the chart of Fig. 8; constants  $K^n$  appear on the upper left-hand scale and constants  $K^m$  on the lower left-hand scale. As in Fig. 7 the horizontal line which intersects the Z-axis is calibrated in degrees from an X-axis, and the lines  $n-n$  and  $m-m$  mark the preferred limits within which a reference W-axis may be selected. The frequency constants  $K^n$  vary from substantially 68.2 for a  $18^\circ$   $W^n$ -angle to substantially 66.6 for a  $29^\circ$   $W^n$ -angle. The frequency constants  $K^m$  vary from substantially 88 for a  $15^\circ$   $W^m$ -angle to substantially 100.6 for a  $29^\circ$   $W^m$ -angle.

The above substantially exact  $K$  values obtain only for quartz piezoelectric elements designed to exhibit a zero temperature coefficient of frequency. The range of frequency constants ( $K^m$  and  $K^n$ ) for crystal-elements designed to exhibit temperature coefficients of frequency other than zero are substantially as follows:

| Temp. coefficient in cycles per million per degree C. | W angles                | Corresponding freq. constant range |
|-------------------------------------------------------|-------------------------|------------------------------------|
| +5                                                    | $W^n=15^\circ-29^\circ$ | $K^n=85$ to $99$ .                 |
| -5                                                    | $W^n=15^\circ-29^\circ$ | $K^n=90$ to $103$ .                |
| +15                                                   | $W^n=13^\circ-29^\circ$ | $K^n=63.6$ to $66.9$ .             |
| -15                                                   | $W^n=13^\circ-29^\circ$ | $K^n=70.2$ to $88.6$ .             |

It will be noted from the chart of Fig. 8 that the constant  $K^m$  for any  $W^m$ -angle is greater than the constant  $K^n$  for the corresponding  $W^n$ -angle. Thus, for the  $20^\circ$  W-angle, constant  $K^n$  is substantially 67.5 whereas the constant  $K^m$  is substantially 95. Since the fundamental frequency of crystal elements of the type described is a function of the thickness dimension, it follows, that the thickness dimension required to achieve a given frequency will be greater when the electrode faces of the element are tilted in a direction towards parallelism with a major apex surface than if these faces are tilted towards parallelism with the plane of a minor apex surface.

Accordingly, and although a finished element having substantially any thickness-frequency and temperature coefficient may be obtained in a blank tilted in either direction, it is recommended that for the relatively higher frequencies (say, above two megacycles) the direction of tilt or rotation about the  $Y+\theta$  axis should be in a direction toward parallelism with the plane of a major apex surface, for when so orientated practical difficulties attendant the cutting and the use of very thin quartz plates are substantially obviated.

Summerizing the data thus far set forth, it will be apparent that before the actual cutting of the element from the mother-crystal commences there are three factors to be considered, to wit:

(1) The thickness-mode frequency at which the finished element is to respond. This factor

determines the frequency constant  $K$  and hence the thickness dimension of the finished element. (As in prior-art "thickness-mode oscillators" the two greater dimensions of crystal elements designed to oscillate at frequencies of two megacycles or higher is unimportant. As in the usual "X-cut" or "Y-cut" "low frequency thickness-mode oscillators" departures from certain known standard length-width ratios and/or electrode surface areas, will alter the oscillating characteristics of the quartz.) The frequency at which the element is to respond will suggest a preferred direction of orientation of the electrode faces of the element with respect to the plane of a major or minor apex surface of the mother-crystal. As above recommended, for relatively high frequencies the electrode surfaces of the blank should preferably, but not necessarily, be rotated (about a  $Y+\theta$  axis) in a direction toward parallelism with the plane of a major apex surface of the mother-crystal.

(2) The temperature coefficient of frequency to be exhibited by the finished element. This factor, like that of frequency, will of course be determined by the use to which the element is to be put. The temperature coefficient of frequency is a function of the angle ( $V$ ) of rotation about a  $Y+\theta$  axis so that it dictates one (the  $V$ ) of the two angles (the  $V$  and  $W$ -angles) necessary to be known.

(3) The relative location of the  $W$ -axis with respect to a reference  $X$ -axis, i. e. the angle ( $W$ ) formed by the intersection of a  $W$ -axis with a reference  $X$ -axis. As previously set forth any  $W$ -angle or axis may be selected within the  $n-n$   $13^{\circ}-29^{\circ}$  range or the  $m-m$   $15^{\circ}-29^{\circ}$  range. (If angles lower than  $13^{\circ}$  and  $15^{\circ}$ , respectively, are chosen the finished element may respond to extra and usually undesired "spurious frequencies.")

As the frequency constant, especially  $K^m$ , increases, the  $W$ -angle increases. The selection of the  $W$ -angle is important only insofar as it is desirable to avoid the use of relatively thin crystal elements. As a matter of manufacturing convenience, it is often desirable to select "standard"  $W$ -angles from the substantially infinite number of  $W$ -angles available. Recommended "standard"  $W$ -angles and their correlated  $V$ -angles and frequency constants ( $K^m$ ,  $K^n$ ) required to achieve a substantially zero and other "low temperature coefficient of frequency" crystals are:

*Tilt towards parallelism with a minor apex face*

| $W^n$ | Temp. coef.=0 |       | Temp. coef.=+15 |       | Temp. coef.=-15 |       |
|-------|---------------|-------|-----------------|-------|-----------------|-------|
|       | $V^n$         | $K^n$ | $V^n$           | $K^n$ | $V^n$           | $K^n$ |
|       |               |       |                 |       |                 |       |
| 60    | 16°           | 34.5  | 67.9            | 29.5  | 68.2            | 40    |
|       | 18°           | 36    | 67.7            | 31    | 68              | 41    |
|       | 20°           | 36.5  | 67.5            | 31.5  | 67.8            | 41.5  |
|       | 25°           | 35.7  | 67              | 30.8  | 67.3            | 40.8  |
|       | 29°           | 35    | 66.6            | 30    | 66.9            | 40    |

*Tilt towards parallelism with a major apex face*

| $W^m$ | Temp. coef.=0 |       | Temp. coef.=+5 |       | Temp. coef.=-5 |       |
|-------|---------------|-------|----------------|-------|----------------|-------|
|       | $V^m$         | $K^m$ | $V^m$          | $K^m$ | $V^m$          | $K^m$ |
|       |               |       |                |       |                |       |
| 70    | 16°           | 27    | 87.5           | 22    | 85.5           | 32    |
|       | 18°           | 37.5  | 92.5           | 32.5  | 90.5           | 42.5  |
|       | 20°           | 43    | 95             | 38    | 93             | 48    |
|       | 25°           | 47    | 99             | 42    | 97             | 52    |
|       | 29°           | 48.5  | 100.6          | 43.5  | 98.5           | 53.5  |

Among the factors not necessary to be considered is whether the mother-crystal is of so called "left-hand quartz" or "right-hand quartz". The system for orientation of the present invention is applicable (without change) to quartz 5 possessing a crystalline structure of either type.

Any  $X$ -axis may be selected as the reference axis from which the  $W$ -axis is measured. This is brought out in the chart of Fig. 9 which shows the characteristics of quartz plates rotated 10 throughout the entire  $360^{\circ}$  scale about the  $Z$ -axis. This chart shows, at a single glance, all of the information required in the planning of a quartz piezoelectric element which shall exhibit a substantially zero temperature coefficient of 15 frequency.

Referring now in detail to Fig. 9, there are three  $X$ -axes and three  $Y$ -axes passing through the  $Z$ -axis and dividing the  $360^{\circ}$  scale into twelve 20  $30^{\circ}$  segments. Each of the substantially infinite 25 number of axes (not marked) between each adjacent  $X$  and  $Y$  axis, in the  $X-Y$  plane, is a  $W$ -axis. As previously set forth preferably only those  $W$ -axes which form  $W$ -angles (with a selected reference,  $X$ -axis) of from substantially 25  $13^{\circ}$  to  $29^{\circ}$  or from substantially  $15^{\circ}$  to  $29^{\circ}$  are employed as reference  $W$ -axes in carrying the invention into effect.

Each  $Y$ -axis bisects four curved lines, designated respectively  $V^m$ ,  $K^m$ ,  $K^n$ ,  $V^n$ . Wherever a 30  $W$ -axis touches one of the curved lines  $V^m$  or  $V^n$ , there is the second or  $V$ -angle of rotation required to be known in the cutting of zero temperature coefficient quartz crystal elements. The scale for reading  $V$ -angles is marked in degrees 35 in two directions along that  $X$ -axis which divides the main  $360^{\circ}$  scale, horizontally. The exponents " $m$ " and " $n$ " are indicative of the direction of tilt with respect to the plane of a major ( $m$ ) and minor ( $n$ ) apex surface of the 40 mother crystal.

The other two curves, i. e.  $K^m$  and  $K^n$  are frequency constant curves. The scale for reading these curves is marked on the lower half of the  $Y$ -axis which extends from the  $90^{\circ}$  main-scale 45 marking through the  $Z$ -axis to the  $270^{\circ}$  marking. As with the case of the  $V^m$  and  $V^n$  curves the exponents " $m$ " and " $n$ " are indicative of the direction of tilt with respect to the plane of a major ( $m$ ) and minor ( $n$ ) apex surface of the 50 mother crystal.

A technician in using the chart of Fig. 9 will first select any "W" angle which intersects the curved  $V$  and  $K$  lines. Assuming, as in the prior example, that the  $W$ -axis selected is  $20^{\circ}$  from an 55  $X$ -axis, then, following the  $20^{\circ}$  line inwardly toward the center of the chart (i. e. toward the  $Z$ -axis) it will be seen that this line intersects line  $V^m$  at "a",  $K^m$  at "b",  $V^m$  at "c" and  $K^m$  at "d". Points "a" and "c" are read on the central 60 horizontal scale and give the precise  $V$ -angle of rotation required for each direction of tilt; i. e. towards a minor apex face ("a") or towards a major apex face ("c"). Projecting points "a" and "c" upon this central scale, it will be seen that if 65 the blank is to be tilted towards a minor apex face the precise angle of tilt required to achieve a zero temperature coefficient of frequency is  $36.5^{\circ}$  and if the blank is to be tilted toward a major apex face,  $43^{\circ}$ .

The frequency constant points "b" and "d" are read on the vertical scale which extends outwardly from the center or  $Z$ -axis of the chart. The frequency constant  $K^n$  for a  $20^{\circ}$   $W^n$ ,  $36.5^{\circ}$   $V^n$  blank when read on this scale is seen to be 67.5 75

and the frequency constant  $K^m$  for a 20 W<sup>m</sup>, 43° V<sup>m</sup> blank is 95.

As illustrative of a preferred manner of cutting piezoelectric elements having a zero or some other low temperature coefficient of frequency reference is had to Figs. 1 to 6 inclusive.

Referring first to Fig. 2, a section 2, say one inch thick, is first sliced from the body of the mother-crystal; the thickness dimension of this 10 section is parallel with, and the length-breadth dimensions normal to the Z-axis. A bar 3 is then cut from this section 2, preferably at substantially the exact W-angle selected as a reference axis. In the illustrated embodiment the 15 long dimensions of the bar 3 coincide with a W-axis which is 20° removed from that X-axis (and hence 10° removed from that Y-axis) marked in Fig. 1.

Referring to Figs. 3 and 4, the blanks 4 and 5 20 from which the finished elements are formed are then sliced from bar 2 at either a V<sup>m</sup> angle or V<sup>n</sup> angle dictated by the temperature coefficient desired. The electrode faces of blank 4, as shown, have been rotated substantially 36.5° (the V<sup>n</sup> 25 angle) about its Y+θ axis in a direction away from parallelism with the Z-axis toward parallelism with the plane of that minor apex surface of the mother-crystal which is designated N<sub>1</sub> in Figs. 1 and 4. (In Fig. 2, N<sub>1</sub> is opposite the major 30 apex surface designated M<sub>1</sub>.) This 36.5 V<sup>n</sup> angle is shown in Figs. 7 and 9 to be the precise angle required to achieve a substantially zero temperature coefficient of frequency—when the selected W-axis forms a W-angle with an X-axis of 20°.

The electrode faces of blank 5 of Figs. 3 and 4 35 have been rotated substantially 48° (the V<sup>m</sup> angle) about its Y+θ axis in a direction away from parallelism with the Z-axis towards parallelism with the plane of that major apex surface of the mother crystal which is designated M<sub>1</sub> in Figs. 1, 2 and 4.

Assuming, for purposes of illustration, that the finished element to be ground or lapped from blank 4 is to respond to a thickness-mode frequency of, say 2 megacycles, then since

$$t \text{ (thickness)} = \frac{K^n}{f} \frac{\text{(frequency constant)}}{\text{(frequency in megacycles)}}$$

50 and K<sup>n</sup> (as shown in Figs. 8 and 9) for a 20° W-angle is equal to substantially 67.5. Therefore,

$$t = \frac{67.5}{2}$$

55 or, solved, t = substantially 33.75 thousandths of an inch.

Assuming, for purposes of illustration, that the finished element to be ground or lapped from blank 5 is to respond to a thickness-mode frequency of, say 8 megacycles. Applying the same formula,

$$t = \frac{95}{8}$$

65 which, solved, shows the thickness dimension required to achieve a 8 megacycle, zero temperature coefficient, V<sup>m</sup> type crystal is substantially 11.875 thousandths of an inch.

70 These dimensions having been determined it remains only to grind and lap the elements to the thickness dimensions set forth and to trim the edges (e, e<sup>1</sup> Fig. 4, e<sup>2</sup> e<sup>3</sup> Fig. 5) so that the thickness dimension W+V, is normal to that one of 75 the greater dimensions of the finished element

which is designated Z+V. It is preferable to bevel the edges and round the corners of the otherwise finished elements of Figs. 4 and 5 in order to remove minute irregularities in the cutting and to prevent chipping in case the crystals should be excited at very great amplitudes of oscillation. As in prior art thickness-mode oscillators and resonators, the shape or configuration of the finished crystal (i. e. whether circular, polygonal, rectangular or other shapes) has little 10 or no effect upon oscillation performance.

Although certain specific ways and means for accomplishing the objects of the invention have been set forth it is to be understood that they have been given for the purpose of explaining the 15 inventive concept and should not be construed as limitations to the scope of the invention. Neither is it to be understood that any statements herein made in regard to the value or 20 relationships between frequency constants, angles of orientation and "temperature coefficients of frequency" are other than close approximations. The invention, therefore, is not to be limited except insofar as is necessitated by the prior art 25 and by the spirit of the appended claims.

What is claimed is:

1. A quartz piezoelectric element cut from a mother crystal having major and minor apex surfaces, said element having an electrode face parallel to a reference plane which is rotated about a Y+θ axis in a direction away from parallelism with the Z-axis and toward parallelism with the plane of one of said apex surfaces, said Y+θ axis being normal to a W-axis which lies at least 1° removed from a Y-axis in a plane normal to the Z-axis, the exact angle formed by the intersection of said reference plane with said Z-axis being determined, in substantial agreement with the chart of Fig. 7, by the temperature coefficient of frequency desired and by the particular apex surface of the mother crystal toward which said electrode face is inclined.

2. A quartz piezoelectric element cut from a mother crystal having major and minor apex surfaces, said element having its electrode faces parallel to a plane which is rotated not less than substantially 14° and no more than substantially 54° about a Y+θ axis in a direction away from parallelism with the Z-axis and toward parallelism with the plane of a major apex surface, said Y+θ axis being normal to a W-axis which lies not less than substantially 15° and no more than substantially 29° removed from an X-axis in a plane normal to the Z-axis.

3. A quartz piezoelectric element cut from a mother crystal having major and minor apex surfaces, said element having its electrode faces parallel to a plane which is rotated from substantially 14° to substantially 54° about a Y+θ axis in a direction away from parallelism with the Z-axis and toward parallelism with the plane of a major apex surface, said Y+θ axis being normal to a W-axis which lies between an X-axis and a Y-axis in a plane normal to the Z-axis, the angle formed by the intersection of said W-axis and said X-axis being between the limits of substantially 15° and not more than 29°, whereby said element exhibits a temperature coefficient of frequency within substantially  $\pm 5$  70 cycles per million per degree centigrade when vibrated at a fundamental thickness-mode frequency.

4. The invention as set forth in claim 3 further characterized in that the thickness of said ele- 75

ment expressed in thousandths of an inch is equal to

$$\frac{K}{f}$$

5 where  $f$  is a fundamental thickness-mode frequency expressed in megacycles and  $K$  is a number of the order of substantially 85 to 103.

10 5. A quartz piezoelectric element cut from a mother crystal having major and minor apex surfaces, said element having its electrode faces parallel to a plane which is rotated from substantially 20° to substantially 49° about a  $Y+\theta$  axis in a direction away from parallelism with the 15 Z-axis and toward parallelism with the plane of a major apex surface, said  $Y+\theta$  axis being normal to a W-axis which lies between an X-axis and a Y-axis in a plane normal to the Z-axis, the angle formed by the intersection of said 20 W-axis and said X-axis being between the limits of substantially 15° and not more than substantially 29°, whereby said element exhibits a substantially zero temperature coefficient of frequency when vibrated at a fundamental thickness-mode frequency.

25 6. The invention as set forth in claim 5 further characterized in that the thickness of said element expressed in thousandths of an inch is equal to

30 
$$\frac{K}{f}$$

where  $f$  is a fundamental thickness-mode frequency expressed in megacycles and  $K$  is a number of the order of substantially 88 to 100.6.

35 7. A quartz piezoelectric element cut from a mother crystal having major and minor apex surfaces, said element having its electrode faces parallel to a plane which is rotated from substantially 14° to substantially 44° about a  $Y+\theta$  axis 40 in a direction away from parallelism with the Z-axis and toward parallelism with the plane of a major apex surface, said  $Y+\theta$  axis being normal to a W-axis which lies between an X-axis and a Y-axis in a plane normal to the Z-axis, the 45 angle formed by the intersection of said W-axis and said X-axis being between the limits of substantially 15° and not more than substantially 29°, whereby said element exhibits a temperature coefficient of frequency of substantially +5 cycles 50 per million per degree centigrade when vibrated at a fundamental thickness-mode frequency.

55 8. The invention as set forth in claim 7 further characterized in that the thickness of said element expressed in thousandths of an inch is equal to

$$\frac{K}{f}$$

60 where  $f$  is a fundamental thickness-mode frequency expressed in megacycles and  $K$  is a number of the order of substantially 85 to 99.

65 9. A quartz piezoelectric element cut from a mother crystal having major and minor apex surfaces, said element having its electrode faces parallel to a plane which is rotated from substantially 25° to substantially 54° about a  $Y+\theta$  axis in a direction away from parallelism with the Z-axis and toward parallelism with the plane of a major apex surface, said  $Y+\theta$  axis being 70 normal to a W-axis which lies between an X-axis and a Y-axis in a plane normal to the Z-axis, the angle formed by the intersection of said W-axis and said X-axis being between the limits of substantially 15° and not more than substantially 29°, whereby said element exhibits a temperature coefficient of frequency of substantially -5 cycles

per million per degree centigrade when vibrated at a fundamental thickness-mode frequency.

10 10. The invention as set forth in claim 9 further characterized in that the thickness of said element expressed in thousandths of an inch is equal to

$$\frac{K}{f}$$

15 where  $f$  is a fundamental thickness-mode frequency expressed in megacycles and  $K$  is a number of the order of substantially 90 to 103.

20 11. A quartz piezoelectric element cut from a mother crystal having major and minor apex surfaces, said element having its electrode faces parallel to a plane which is rotated not less than substantially 27° and no more than substantially 42° about a  $Y+\theta$  axis in a direction away from parallelism with the Z-axis and toward parallelism with the plane of a minor apex surface, said  $Y+\theta$  axis being normal to a W-axis which lies not less than substantially 13° and no more than substantially 29° removed from an X-axis in a plane normal to the Z-axis.

25 12. A quartz piezoelectric element cut from a mother crystal having major and minor apex surfaces, said element having its electrode faces parallel to a plane which is rotated from substantially 27° to substantially 42° about a  $Y+\theta$  axis in a direction away from parallelism with the Z-axis and toward parallelism with the plane of a minor apex surface, said  $Y+\theta$  axis being normal to a W-axis which lies between an X-axis and a Y-axis in a plane normal to the Z-axis, the angle formed by the intersection of said W-axis and said X-axis being between the limits of substantially 13° and not more than substantially 29°, whereby said element exhibits a temperature coefficient of frequency within substantially  $\pm 15$  cycles per million per degree centigrade when vibrated at a fundamental thickness-mode frequency.

30 13. The invention as set forth in claim 12 further characterized in that the thickness of said element expressed in thousandths of an inch is equal to

$$\frac{K}{f}$$

35 where  $f$  is a fundamental thickness-mode frequency expressed in megacycles and  $K$  is a number of the order of substantially 70.2 to 66.9.

40 14. A quartz piezoelectric element cut from a mother crystal having major and minor apex surfaces, said element having its electrode faces parallel to a plane which is rotated from substantially 32° to substantially 37° about a  $Y+\theta$  axis in a direction away from parallelism with the Z-axis and toward parallelism with the plane of a minor apex surface, said  $Y+\theta$  axis being normal to a W-axis which lies between an X-axis and a Y-axis in a plane normal to the Z-axis, the angle formed by the intersection of said W-axis and said X-axis being between the limits of substantially 13° and not more than substantially 29°, whereby said element exhibits a substantially zero temperature coefficient of frequency when vibrated at a fundamental thickness-mode frequency.

45 15. The invention as set forth in claim 14 further characterized in that the thickness of said element expressed in thousandths of an inch is equal to

$$\frac{K}{f}$$

50 where  $f$  is a fundamental thickness-mode frequency.

quency expressed in megacycles and  $K$  is a number of the order of substantially 68.2 to 66.6.

16. A quartz piezoelectric element cut from a mother crystal having major and minor apex surfaces, said element having its electrode faces parallel to a plane which is rotated from substantially  $27^\circ$  to substantially  $32^\circ$  about a  $Y+\theta$  axis in a direction away from parallelism with the  $Z$ -axis and toward parallelism with the plane 10 of a minor apex surface, said  $Y+\theta$  axis being normal to a  $W$ -axis which lies between an  $X$ -axis and a  $Y$ -axis in a plane normal to the  $Z$ -axis, the angle formed by the intersection of said  $W$ -axis and said  $X$ -axis being between the limits 15 of substantially  $13^\circ$  and not more than substantially  $29^\circ$ , whereby said element exhibits a temperature coefficient of frequency of substantially  $+15$  cycles per million per degree centigrade when vibrated at a fundamental thickness mode 20 frequency.

17. The invention as set forth in claim 16 further characterized in that the thickness of said element expressed in thousandths of an inch is equal to

$$\frac{K}{f}$$

where  $f$  is a fundamental thickness-mode frequency expressed in megacycles and  $K$  is a number of the order of substantially 68.6 to 66.9.

18. A quartz piezoelectric element cut from a mother crystal having major and minor apex surfaces, said element having its electrode faces parallel to a plane which is rotated from substantially  $37^\circ$  to substantially  $42^\circ$  about a  $Y+\theta$  axis in a direction away from parallelism with the  $Z$ -axis and toward parallelism with the plane of a minor apex surface, said  $Y+\theta$  axis being normal to a  $W$ -axis which lies between an  $X$ -axis and a  $Y$ -axis in a plane normal to the  $Z$ -axis, the angle formed by the intersection of said  $W$ -axis and said  $X$ -axis being between the limits of substantially  $13^\circ$  and not more than substantially  $29^\circ$ , whereby said element exhibits a temperature coefficient of frequency of sub-

stantially  $-15$  cycles per million per degree centigrade when vibrated at a fundamental thickness-mode frequency.

19. The invention as set forth in claim 18 further characterized in that the thickness of said element expressed in thousandths of an inch is equal to

$$\frac{K}{f}$$

10

where  $f$  is a fundamental thickness-mode frequency expressed in megacycles and  $K$  is a number of the order of substantially 70.2 to 68.6.

20. A quartz piezoelectric element of low temperature coefficient of frequency adapted to vibrate in a shear mode at a frequency determined substantially by its thickness or smallest dimension which is perpendicular to its substantially parallel major surfaces, said major surfaces having an edge axis inclined substantially 20  $90^\circ$  with respect to the  $Z$  axis and substantially  $10^\circ$  degrees with respect to an  $X$  axis, and having another edge axis disposed substantially perpendicular to said first-mentioned edge axis and inclined with respect to the  $Z$  axis substantially  $+36^\circ$  degrees or toward parallelism with the plane of a minor apex face of the crystal from which said element is cut.

21. A quartz piezoelectric element of low temperature coefficient of frequency adapted to vibrate in a shear mode at a frequency determined substantially by its thickness or smallest dimension which is perpendicular to its substantially parallel major surfaces, said major surfaces having an edge axis inclined substantially  $90^\circ$  with respect to the  $Z$  axis and substantially  $5^\circ$  with respect to an  $X$  axis, and having another edge axis disposed substantially perpendicular to said first-mentioned edge axis and inclined with respect to the  $Z$  axis substantially  $+35.5^\circ$  or toward parallelism with the plane of a minor apex face of the crystal from which said element is cut.

CHARLES F. BALDWIN.  
SAMUEL A. BOKOVY.

45